



US009502170B2

(12) **United States Patent**  
**Odahara**

(10) **Patent No.:** **US 9,502,170 B2**  
(45) **Date of Patent:** **Nov. 22, 2016**

(54) **ELECTRONIC COMPONENT AND METHOD  
FOR PRODUCING SAME**

(71) Applicant: **MURATA MANUFACTURING CO., LTD.**, Kyoto (JP)

(72) Inventor: **Mitsuru Odahara**, Kyoto-fu (JP)

(73) Assignee: **Murata Manufacturing Co., Ltd.**, Kyoto (JP)

(\*) Notice: Subject to any disclaimer, the term of this patent is extended or adjusted under 35 U.S.C. 154(b) by 341 days.

(21) Appl. No.: **14/087,771**

(22) Filed: **Nov. 22, 2013**

(65) **Prior Publication Data**

US 2014/0078643 A1 Mar. 20, 2014

**Related U.S. Application Data**

(63) Continuation of application No. PCT/JP2012/063128, filed on May 23, 2012.

(30) **Foreign Application Priority Data**

Jun. 15, 2011 (JP) ..... 2011-133196

(51) **Int. Cl.**

**H01G 4/30** (2006.01)

**H01G 4/005** (2006.01)

**H01G 4/228** (2006.01)

**H01F 27/29** (2006.01)

**H01F 17/00** (2006.01)

(52) **U.S. Cl.**

CPC ..... **H01F 27/29** (2013.01); **H01F 17/0013** (2013.01); **H01F 27/292** (2013.01)

(58) **Field of Classification Search**

CPC ..... H01G 4/30

USPC ..... 361/301.4, 303, 306.1, 306.3; 29/25.42  
See application file for complete search history.

(56) **References Cited**

**U.S. PATENT DOCUMENTS**

6,715,197 B2 \* 4/2004 Okuyama ..... H01F 17/0013  
29/592.1  
7,075,775 B2 \* 7/2006 Yamazaki ..... H01C 1/02  
338/237

(Continued)

**FOREIGN PATENT DOCUMENTS**

CN 101228601 A 7/2008  
JP 2002-367833 A 12/2002

(Continued)

**OTHER PUBLICATIONS**

International Search Report; PCT/JP2012/063128; Aug. 14, 2012.  
(Continued)

*Primary Examiner* — Eric Thomas

(74) *Attorney, Agent, or Firm* — Studebaker & Brackett  
PC

(57) **ABSTRACT**

An electronic component comprises: a laminate having a plurality of rectangular insulator layers and a mounting surface formed by a series of sides of the insulator layers. A plurality of first lead-out conductors are exposed between the insulator layers at the mounting surface. A first external electrode covers the first lead-out conductors at the mounting surface. The first external electrode is located at a first formation area at the mounting surface. The first formation area, when viewed in a plan view in an extending direction in which the sides of the insulator layers that constitute the mounting surface extend, is curved so as to bulge at a center of the formation area relative to opposite ends thereof.

**20 Claims, 12 Drawing Sheets**



---

|                          |                         |                         |                                                                                                                                                                                                                                                                  |
|--------------------------|-------------------------|-------------------------|------------------------------------------------------------------------------------------------------------------------------------------------------------------------------------------------------------------------------------------------------------------|
| (56)                     | <b>References Cited</b> | JP                      | 5668849 B2 2/2015                                                                                                                                                                                                                                                |
| <hr/>                    |                         |                         |                                                                                                                                                                                                                                                                  |
| U.S. PATENT DOCUMENTS    |                         |                         |                                                                                                                                                                                                                                                                  |
| 7,633,739 B2 *           | 12/2009 Devoe .....     | H01G 4/232<br>361/306.3 | Written Opinion of the International Searching Authority; PCT/JP2012/063128; Aug. 14, 2012.                                                                                                                                                                      |
| 7,995,326 B2 *           | 8/2011 Ueda .....       | H01C 1/142<br>361/306.1 | An Office Action; "Decision of Refusal," issued by the Japanese Patent Office on Aug. 19, 2014, which corresponds to Japanese Patent Application No. 2013-520488 and is related to U.S. Appl. No. 14/087,771; with English language translation.                 |
| 2008/0128860 A1          | 6/2008 Sawada et al.    | H01G 4/012<br>361/303   | An Office Action; "Notification of Reasons for Refusal," issued by the Japanese Patent Office on Jan. 7, 2014, which corresponds to Japanese Patent Application No. 2013-520488 and is related to U.S. Appl. No. 14/087,771; with English language translation.  |
| 2010/0085682 A1 *        | 4/2010 Abe .....        | H01G 4/012<br>361/303   | An Office Action; "Notification of Reasons for Refusal," issued by the Japanese Patent Office on Jun. 14, 2016, which corresponds to Japanese Patent Application No. 2014-213720 and is related to U.S. Appl. No. 14/087,771; with English language translation. |
| 2014/0078643 A1          | 3/2014 Odahara          |                         |                                                                                                                                                                                                                                                                  |
| FOREIGN PATENT DOCUMENTS |                         |                         |                                                                                                                                                                                                                                                                  |
| JP                       | 2004-200373 A           | 7/2004                  |                                                                                                                                                                                                                                                                  |
| JP                       | 2005-322743 A           | 11/2005                 |                                                                                                                                                                                                                                                                  |
| JP                       | 2006-114626 A           | 4/2006                  |                                                                                                                                                                                                                                                                  |
| JP                       | 2006-237078 A           | 9/2006                  |                                                                                                                                                                                                                                                                  |
| JP                       | 2007-096215 A           | 4/2007                  |                                                                                                                                                                                                                                                                  |
| JP                       | 2009-111314 A           | 5/2009                  |                                                                                                                                                                                                                                                                  |
| JP                       | 2010-080703 A           | 4/2010                  |                                                                                                                                                                                                                                                                  |

\* cited by examiner

FIG. 1 A



FIG. 1 B



FIG. 1 C



FIG. 2



FIG. 3 A

12

FIG. 3 B

10

FIG. 4



FIG. 5



F I G . 6 A



F I G . 6 B



F 1 G. 7



FIG. 8



FIG. 9



FIG. 10 A

12

FIG. 10 B

10d

FIG. 11 A



FIG. 11 B



FIG. 11 C



## F I G . 1 2



FIG. 13 A



FIG. 13 B



FIG. 14.

FIG. 15  
PRIOR ART

## 1

ELECTRONIC COMPONENT AND METHOD  
FOR PRODUCING SAMECROSS REFERENCE TO RELATED  
APPLICATIONS

This application claims benefit of priority to Japanese Patent Application No. 2011-133196 filed on Jun. 15, 2011, and to International Patent Application No. PCT/JP2012/063128 filed on May 23, 2012, the entire content of each of which is incorporated herein by reference.

## TECHNICAL FIELD

The present disclosure relates to electronic components and methods for producing the same, more particularly to an electronic component including a laminate formed by laminating insulator layers and a method for producing the same.

## BACKGROUND

As a conventional electronic component, a laminated coil component described in, for example, Japanese Patent Laid-Open Publication No. 2005-322743 is known. FIG. 15 is a transparent view of the laminated coil component 100 described in Japanese Patent Laid-Open Publication No. 2005-322743.

The laminated coil component 100 includes a ceramic laminate 110, a coil conductor 120, and a set of external electrodes 130. The ceramic laminate 110 is formed by laminating a plurality of ceramic layers. The coil conductor 120 is a helical coil formed by connecting inner conductor layers 121 and via holes 122 in series, so as to have a coil axis parallel to the direction of lamination of the ceramic laminate 110. Each of the external electrodes 130 is provided on a mounting surface positioned in a direction perpendicular to the direction of lamination, and is connected to either end of the coil conductor 120. The laminated coil component 100 thus configured is mounted onto a circuit board by soldering the external electrodes 130 onto lands of the circuit board. However, the laminated coil component 100 described in Japanese Patent Laid-Open Publication No. 2005-322743 might have air left trapped in the solder. More specifically, the external electrodes 130 are provided only on the mounting surface and in the form of flat plates. When the laminated coil component 100 is mounted onto the circuit board, if air is trapped in the solder, it is caught between the external electrodes 130 and the lands, so that it cannot escape from the solder. In this manner, when air remains in the solder, there might be poor connections between the lands and the external electrodes 130.

## SUMMARY

The present disclosure provides an electronic component capable of reducing poor connection between a land and an external electrode and a method for producing the same.

An electronic component according to one embodiment of the present disclosure includes: a laminate having a plurality of rectangular insulator layers and a mounting surface formed by a series of sides of the insulator layers; a plurality of first lead-out conductors exposed between the insulator layers at the mounting surface; and a first external electrode covering the first lead-out conductors at the mounting surface, the first external electrode being located at a first formation area at the mounting surface, the first formation area, when viewed in a plan view in an extending direction

## 2

in which the sides of the insulator layers that constitute the mounting surface extend, is curved so as to bulge at a center of the first formation area relative to opposite ends thereof. Further, the other embodiment of the present disclosure is directed to a method for producing an electronic component, the electronic component including a laminate having a plurality of rectangular insulator layers and a mounting surface formed by a series of sides of the insulator layers; a plurality of first lead-out conductors exposed between the insulator layers at the mounting surface; and a first external electrode covering the first lead-out conductors at the mounting surface, the first external electrode being located at a first formation area at the mounting surface, and the first formation area, when viewed in a plan view in an extending direction in which the sides of the insulator layers that constitute the mounting surface extend, being curved so as to bulge at a center of the first formation area relative to opposite ends thereof, and a circuit element including a plurality of conductive members. The method of the other embodiment of the present disclosure includes the steps of: obtaining the laminate in an unsintered state, the laminate being provided with the first lead-out conductors and the conductive members; and firing the laminate.

## BRIEF DESCRIPTION OF THE DRAWINGS

FIGS. 1A, 1B, and 1C are plan views of an electronic component according to an exemplary embodiment of the disclosure

FIG. 2 is an exploded view of a laminate in the electronic component of FIG. 1.

FIG. 3A is an external oblique view of the laminate in the electronic component of FIG. 1.

FIG. 3B is an external oblique view of the electronic component of FIG. 1.

FIG. 4 is a cross-sectional structure view taken along line X-X of FIG. 3A.

FIG. 5 is a diagram illustrating an electronic component mounted on a circuit board.

FIGS. 6A and 6B are diagrams each illustrating the electronic component sucked by a nozzle.

FIG. 7 is a cross-sectional structure view of an electronic component according to a first exemplary modification.

FIG. 8 is a cross-sectional structure view of an electronic component according to a second exemplary modification.

FIG. 9 is a cross-sectional structure view of an electronic component according to a third exemplary modification.

FIG. 10A is an external oblique view of a laminate in an electronic component according to a fourth exemplary modification.

FIG. 10B is an external oblique view of the electronic component according to the fourth exemplary modification.

FIGS. 11A, 11B, and 11C are plan views of an electronic component according to a fifth exemplary modification.

FIG. 12 is an exploded view of a laminate in the electronic component according to the fifth exemplary modification.

FIG. 13A is an external oblique view of the laminate in the electronic component according to the fifth exemplary modification.

FIG. 13B is an external oblique view of the electronic component according to the fifth exemplary modification.

FIG. 14 is a cross-sectional structure view taken along line X-X of FIG. 13A.

FIG. 15 is a perspective view of a laminated coil component described in Japanese Patent Laid-Open Publication No. 2005-322743.

## DETAILED DESCRIPTION

Hereinafter, an electronic component according to an embodiment of the present disclosure and a method for producing the same will be described.

**Configuration of Electronic Component:** The electronic component according to one exemplary embodiment of the present disclosure will now be described with reference to the drawings. FIGS. 1A, 1B, and 1C are plan views of the electronic component 10 according to the embodiment. FIG. 2 is an exploded view of a laminate 12 in the electronic component 10 of FIG. 1. FIG. 3A is an external oblique view of the laminate 12 in the electronic component 10 of FIG. 1. FIG. 3B is an external oblique view of the electronic component 10 of FIG. 1. FIG. 4 is a cross-sectional structure view taken along line X-X of FIG. 3A. In FIG. 4, external electrodes 14a and 14b are not shown. In the following, the direction of lamination of the electronic component 10 will be defined as a y-axis direction, and the direction along a short side of the electronic component 10 in a plan view in the y-axis direction will be defined as a z-axis direction, and the direction along a long side of the electronic component 10 in a plan view in the y-axis direction will be defined as an x-axis direction. The x-, y- and z-axes are perpendicular to one another.

The electronic component 10 includes the laminate 12, the external electrodes 14a and 14b, dummy lead-out conductors 20a to 20g and 24a to 24g, lead-out conductors 22 and 26, a coil L, and via-hole conductors v11 to v24, as shown in FIGS. 1A, 1B, 1C, and 2.

The laminate 12 is in the shape of a rectangular solid, and has the coil L provided therein. The laminate 12 has a bottom surface S1, a top surface S2, side surfaces S3 and S4, and end surfaces S5 and S6. The bottom surface S1 is a surface of the laminate 12 on the negative side in the z-axis direction, and serves as a mounting surface to face a circuit board when the electronic component 10 is mounted on the circuit board. The top surface S2 is a surface of the laminate 12 on the positive side in the z-axis direction. The side surface S3 is a surface of the laminate 12 on the negative side in the y-axis direction. The side surface S4 is a surface of the laminate 12 on the positive side in the y-axis direction. The end surface S5 is a surface of the laminate 12 on the negative side in the x-axis direction. The end surface S6 is a surface of the laminate 12 on the positive side in the x-axis direction.

The laminate 12 is formed by laminating insulator layers 16a to 16j in this order, from the negative side toward the positive side in the y-axis direction, as shown in FIG. 2. Each of the insulator layers 16a to 16j has a rectangular shape, and is made of, for example, a Ni—Cu—Zn ferrite magnetic material. In the following, the surfaces of the insulator layers 16a to 16j on the negative side in the y-axis direction will be referred to as the front faces, and the surfaces of the insulator layers 16a to 16j on the positive side in the y-axis direction will be referred to as the back faces.

The bottom surface S1 is formed by a series of the long sides of the insulator layers 16a to 16j on the negative side in the z-axis direction. The top surface S2 is formed by a series of the long sides of the insulator layers 16a to 16j on the positive side in the z-axis direction. The side surface S3 is formed by the front face of the insulator layer 16a. The side surface S4 is formed by the back face of the insulator layer 16j. The end surface S5 is formed by a series of the short sides of the insulator layers 16a to 16j on the negative side in the x-axis direction. The end surface S6 is formed by

a series of the short sides of the insulator layers 16a to 16j on the positive side in the x-axis direction.

The coil L includes coil conductors 18a to 18d and via-hole conductors v1 to v3, as shown in FIG. 2. The coil L is a helical coil formed by connecting the coil conductors 18a to 18d by the via-hole conductors v1 to v3. The coil L has a coil axis extending in the y-axis direction, and winds clockwise toward the negative side in the y-axis direction in a plan view from the negative side in the y-axis direction. Moreover, the coil L has terminals t1 and t2. The terminal t1 of the coil L is positioned on the positive side in the y-axis direction relative to the terminal t2.

The coil conductors 18a to 18d are provided on the insulator layers 16d to 16g, respectively, as shown in FIG. 2. Each of the coil conductors 18a to 18d is made of an Ag-based conductive material, and is a linear conductor curved so as to constitute a part of an ellipse. The coil conductors 18a to 18d overlap one another to form an ellipse in a plan view in the y-axis direction. In the following, the ends of the coil conductors 18a to 18d that are located upstream in the clockwise direction will be simply referred to as the upstream ends, and the ends of the coil conductors 18a to 18d that are located downstream in the clockwise direction will be simply referred to as the downstream ends. The terminal t1 of the coil L is at the upstream end of the coil conductor 18d, and the terminal t2 of the coil L is at the downstream end of the coil conductor 18a.

The via-hole conductors v1 to v3 connect the coil conductors 18a to 18d. More specifically, the via-hole conductor v1 connects the upstream end of the coil conductor 18a to the downstream end of the coil conductor 18b. The via-hole conductor v2 connects the upstream end of the coil conductor 18b to the downstream end of the coil conductor 18c. The via-hole conductor v3 connects the upstream end of the coil conductor 18c to the downstream end of the coil conductor 18d.

The lead-out conductor 22 is provided on the front face of the insulator layer 16g, so as to be exposed between the insulator layers 16f and 16g at the bottom surface S1. More specifically, the lead-out conductor 22 has a rectangular shape extending in the x-axis direction and provided along the long side of the insulator layer 16g on the negative side in the z-axis direction. The lead-out conductor 22 is positioned near the end of the long side of the insulator layer 16g that is positioned on the negative side in the z-axis direction and on the positive side in the x-axis direction, and the lead-out conductor 22 is not in contact with the short side of the insulator layer 16g on the positive side in the x-axis direction. As a result, the lead-out conductor 22 is exposed at the bottom surface S1 as a linear strip extending in the x-axis direction. Moreover, the lead-out conductor 22 is connected to the upstream end of the coil conductor 18d.

The dummy lead-out conductors 20a to 20g are provided on the front faces of the insulator layers 16b to 16f, 16h, and 16i, respectively, so as to be exposed between the insulator layers 16a to 16g at the bottom surface S1. The dummy lead-out conductors 20a to 20g have the same shape as the lead-out conductor 22, and are aligned in an entirely overlapping manner in a plan view in the y-axis direction. As a result, the lead-out conductor 22 and the dummy lead-out conductors 20a to 20g are exposed within a rectangular formation area A1 at the bottom surface S1, as shown in FIG. 3A.

The lead-out conductor 22 and the dummy lead-out conductors 20a to 20g are thicker than the coil conductors 18a to 18d, as shown in FIG. 4.

Furthermore, the dummy lead-out conductors **20a** and **20b** and the dummy lead-out conductors **20f** and **20g** are provided outside in the y-axis direction (i.e., either on the positive side or the negative side in the y-axis direction) relative to the terminals **t1** and **t2** of the coil **L**.

The lead-out conductor **26** is provided on the front face of the insulator layer **16d**, so as to be exposed between the insulator layers **16c** and **16d** at the bottom surface **S1**. More specifically, the lead-out conductor **26** has a rectangular shape extending in the x-axis direction and provided along the long side of the insulator layer **16d** on the negative side in the z-axis direction. The lead-out conductor **26** is positioned near the end of the long side of the insulator layer **16d** that is positioned on the negative side in the z-axis direction and on the negative side in the x-axis direction, and the lead-out conductor **26** is not in contact with the short side of the insulator layer **16d** on the negative side in the x-axis direction. As a result, the lead-out conductor **26** is exposed at the bottom surface **S1** as a linear strip extending in the x-axis direction. Moreover, the lead-out conductor **26** is connected to the downstream end of the coil conductor **18a**.

The dummy lead-out conductors **24a** to **24g** are provided on the front faces of the insulator layers **16b**, **16c**, and **16e** to **16i**, respectively, so as to be exposed between the insulator layers **16a** to **16g** at the bottom surface **S1**. The dummy lead-out conductors **24a** to **24g** have the same shape as the lead-out conductor **26**, and are aligned in an entirely overlapping manner in a plan view in the y-axis direction. As a result, the lead-out conductor **26** and the dummy lead-out conductors **24a** to **24g** are exposed within a rectangular formation area **A2** at the bottom surface **S1**, as shown in FIG. 3A.

The lead-out conductor **26** and the dummy lead-out conductors **24a** to **24g** are thicker than the coil conductors **18a** to **18d**.

Furthermore, the dummy lead-out conductors **24a** and **24b** and the dummy lead-out conductors **24f** and **24g** are provided outside in the y-axis direction (i.e., either on the positive side or the negative side in the y-axis direction) relative to the terminals **t1** and **t2** of the coil **L**.

The via-hole conductors **v11** to **v17** are provided so as to pierce through the insulator layers **16b** to **16h**, respectively, in the y-axis direction, and overlap one another in a plan view in the y-axis direction. The via-hole conductor **v11** connects the dummy lead-out conductors **20a** and **20b**. The via-hole conductor **v12** connects the dummy lead-out conductors **20b** and **20c**. The via-hole conductor **v13** connects the dummy lead-out conductors **20c** and **20d**. The via-hole conductor **v14** connects the dummy lead-out conductors **20d** and **20e**. The via-hole conductor **v15** connects the dummy lead-out conductor **20e** and the lead-out conductor **22**. The via-hole conductor **v16** connects the lead-out conductor **22** and the dummy lead-out conductor **20f**. The via-hole conductor **v17** connects the dummy lead-out conductors **20f** and **20g**. As a result, the lead-out conductor **22** and the dummy lead-out conductors **20a** to **20g** are connected.

The via-hole conductors **v18** to **v24** are provided so as to pierce through the insulator layers **16b** to **16h**, respectively, in the y-axis direction, and overlap one another in a plan view in the y-axis direction. The via-hole conductor **v18** connects the dummy lead-out conductors **24a** and **24b**. The via-hole conductor **v19** connects the dummy lead-out conductor **24b** and the lead-out conductor **26**. The via-hole conductor **v20** connects the lead-out conductor **26** and the dummy lead-out conductor **24c**. The via-hole conductor **v21** connects the dummy lead-out conductors **24c** and **24d**. The via-hole conductor **v22** connects the dummy lead-out con-

ductors **24d** and **24e**. The via-hole conductor **v23** connects the dummy lead-out conductors **24e** and **24f**. The via-hole conductor **v24** connects the dummy lead-out conductors **24f** and **24g**. As a result, the lead-out conductor **26** and the dummy lead-out conductors **24a** to **24g** are connected.

The external electrode **14a** is formed by directly plating the formation area **A1** at the bottom surface **S1** of the laminate **12**, so as to cover the dummy lead-out conductors **20a** to **20g** and the lead-out conductor **22** at the bottom surface **S1**, as shown in FIG. 3B. The external electrode **14b** is formed by directly plating the formation area **A2** at the bottom surface **S1** of the laminate **12**, so as to cover the dummy lead-out conductors **24a** to **24g** and the lead-out conductor **26** at the bottom surface **S1**, as shown in FIG. 3B. The external electrodes **14a** and **14b** have the same rectangular shape as the formation areas **A1** and **A2**, respectively, and do not extend to the side surfaces **S3** and **S4** and the end surfaces **S5** and **S6**, which are adjacent to the bottom surface **S1**. Moreover, the external electrode **14a** is positioned on the positive side in the x-axis direction relative to the external electrode **14b**. Examples of the materials of the external electrodes **14a** and **14b** include Cu, Ni, and Sn.

The electronic component **10** thus configured has features as will be described below, in the cross section shown in FIG. 4, which is normal to the x-axis direction and includes the lead-out conductor **22**, the dummy lead-out conductors **20a** to **20g**, and the coil conductors **18a** to **18d**. First, a portion of the cross section that includes the lead-out conductor **22** and the dummy lead-out conductors **20a** to **20g** will be referred to as a cross-sectional region **E1**. The rest of the cross section other than the cross-sectional region **E1**, which includes the coil conductors **18a** to **18d**, will be referred to as a cross-sectional region **E2**. The cross-sectional region **E1** is a region between the bottom surface **S1** and a line **L1** parallel to the y-axis and dividing the dummy lead-out conductors **20a** to **20g** and the lead-out conductor **22** from the coil conductors **18a** to **18d**. The cross-sectional region **E2** is a region between the top surface **S2** and the line **L1**.

As shown in FIG. 4, the proportion of an area occupied by the lead-out conductor **22** and the dummy lead-out conductors **20a** to **20g** in the cross-sectional region **E1** is greater than the proportion of an area occupied by the coil conductors **18a** to **18d** in the cross-sectional region **E2**.

Furthermore, in a cross section not shown in the figure, a portion of the cross section that includes the lead-out conductor **26** and the dummy lead-out conductors **24a** to **24g** will be referred to as a cross-sectional region **E1**. The rest of the cross section other than the cross-sectional region **E1**, which includes the coil conductors **18a** to **18d**, will be referred to as a cross-sectional region **E2**. The cross-sectional region **E1** is a region between the bottom surface **S1** and a line **L1** extending on the positive side in the z-axis direction relative to a line connecting the ends of the dummy lead-out conductors **24a** to **24g** and the lead-out conductor **26** on the positive side in the z-axis direction. The cross-sectional region **E2** is a region between the top surface **S2** and the line **L1**.

The proportion of an area occupied by the lead-out conductor **26** and the dummy lead-out conductors **24a** to **24g** in the cross-sectional region **E1** is greater than the proportion of an area occupied by the coil conductors **18a** to **18d** in the cross-sectional region **E2**.

Furthermore, in the electronic component **10**, the formation areas **A1** and **A2**, when viewed in a plan view in an extended direction (x-axis direction) in which the long sides of the insulator layers **16a** to **16j** that constitute the bottom

surface S1 extend, are curved so as to bulge at the center toward the negative side in the z-axis direction relative to the opposite ends, as shown in FIG. 4. In the electronic component 10 according to the present embodiment, the bottom surface S1, when viewed in a plan view in the x-axis direction, is curved so as to bulge at the center toward the negative side in the z-axis direction relative to the opposite ends. The amount of curving D of the bottom surface S1 refers to the distance in the z-axis direction from the level of the most bulging point of the bottom surface S1 (typically, the center of the bottom surface S1 in the y-axis direction) to the level of the opposite ends of the bottom surface S1 in the y-axis direction, as shown in FIG. 4.

Furthermore, the external electrodes 14a and 14b are provided in the formation areas A1 and A2, respectively. Therefore, the external electrodes 14a and 14b, when viewed in a plan view in the x-axis direction, are also curved so as to bulge at the center toward the negative side in the z-axis direction relative to the opposite ends.

**Method for Producing Electronic Component:** The method for producing the electronic component 10 will be described below with reference to the drawings. Note that in the method described below, a plurality of electronic components 10 are produced simultaneously.

Initially, ceramic green sheets from which to make insulator layers 16a to 16j of FIG. 2 are prepared. Specifically, materials weighed at a predetermined ratio, including ferric oxide ( $Fe_2O_3$ ), zinc oxide (ZnO), copper oxide (CuO), and nickel oxide (NiO), are introduced into a ball mill as raw materials, and subjected to wet mixing. The resultant mixture is dried and ground to obtain powder, which is pre-sintered at 800° C. for 1 hour. The resultant pre-sintered powder is subjected to wet grinding in the ball mill, and thereafter dried and cracked to obtain ferrite ceramic powder having an average grain size of 2  $\mu m$ .

To the ferrite ceramic powder, a binder (vinyl acetate, water-soluble acrylic, or the like), a plasticizer, a wetting agent, and a dispersing agent are added and mixed in the ball mill, and thereafter defoamed under reduced pressure. The resultant ceramic slurry is spread over carrier sheets by a doctor blade method and dried to form ceramic green sheets from which to make insulator layers 16a to 16j.

Next, via-hole conductors v1 to v24 are provided through their respective ceramic green sheets from which to make insulator layers 16b to 16h. Specifically, the ceramic green sheets from which to make insulator layers 16b to 16h are irradiated with laser beams to bore via holes therethrough. In addition, a paste made of a conductive material such as Ag, Pd, Cu, Au, or an alloy thereof, is applied by printing or suchlike to fill the via holes.

Next, coil conductors 18a to 18d, dummy lead-out conductors 20a to 20g and 24a to 24g, and lead-out conductors 22 and 26 are formed in the principal surfaces (hereinafter, referred to as the front faces) of the ceramic green sheets from which to make insulator layers 16b to 16i, on the negative side in the z-axis direction, as shown in FIG. 2. Specifically, a conductive paste mainly composed of Ag, Pd, Cu, Au, or an alloy thereof is applied by screen printing or photolithography onto the front faces of the ceramic green sheets from which to make insulator layers 16b to 16i, thereby forming the coil conductors 18a to 18d, the dummy lead-out conductors 20a to 20g and 24a to 24g, and the lead-out conductors 22 and 26. Note that forming the coil conductors 18a to 18d, the dummy lead-out conductors 20a to 20g and 24a to 24g, and the lead-out conductors 22 and 26 and filling the via holes with the conductive paste may be included in the same step.

Next, the ceramic green sheets from which to make insulator layers 16a to 16j are laminated in this order, as shown in FIG. 2, and then subjected to pressure-bonding, thereby obtaining an unsintered mother laminate. In the lamination and the pressure-bonding of the ceramic green sheets from which to make insulator layers 16a to 16j, the sheets are laminated one by one and then subjected to pressure-bonding to obtain the unsintered mother laminate, and thereafter, the mother laminate is firmly bonded by 10 pressing with an isostatic press or suchlike.

Next, the mother laminate is cut by a cutter into a predetermined size, thereby obtaining unsintered laminates 12. Each of the unsintered laminates 12 is subjected to debinding and sintering. The debinding is performed, for example, in a low-oxygen atmosphere at 500° C. for two hours. The sintering is performed, for example, at 800° C. to 900° C. for 2.5 hours.

During the sintering, the insulator layers 16a to 16j, the coil conductors 18a to 18d, the dummy lead-out conductors 20a to 20g and 24a to 24g, and the lead-out conductors 22 and 26 contract. The degree of contraction of the insulator layers 16a to 16j, which are made of ceramic, is greater than the degree of contraction of the coil conductors 18a to 18d, the dummy lead-out conductors 20a to 20g and 24a to 24g, and the lead-out conductors 22 and 26, which are made of conductive materials. Therefore, the cross-sectional region E2, which has a relatively small proportion of conductive material, contracts more than the cross-sectional region E1, which has a relatively large proportion of conductive material. Accordingly, the width of the cross-sectional region E2 in the y-axis direction is less than the width of the cross-sectional region E1 in the y-axis direction, as shown in FIG. 4. Therefore, the opposite ends of the cross-sectional region E2 in the y-axis direction are pulled upward in the z-axis direction. As a result, the bottom surface S1 is curved so as to bulge at the center toward the negative side in the z-axis direction relative to the opposite ends.

Next, the laminate 12 is barreled for beveling, and plated with Ni and Sn, thereby forming external electrodes 14a and 14b. Specifically, the dummy lead-out conductors 20a to 20g and 24a to 24g, and the lead-out conductors 22 and 26 are exposed from the bottom surface S1 of the laminate 12. Accordingly, conductive films are grown from the dummy lead-out conductors 20a to 20g and 24a to 24g, and the lead-out conductors 22 and 26 by a plating method, thereby forming the external electrodes 14a and 14b, as shown in FIG. 3B. By the foregoing process, the electronic component 10 as shown in FIG. 1 is completed.

**Effects:** The electronic component 10 according to the present embodiment renders it possible to inhibit air from being left trapped in the solder that connects the lands of the circuit board to the external electrodes 14a and 14b. More specifically, the laminated coil component 100 described in Japanese Patent Laid-Open Publication No. 2005-322743 has the external electrodes 130 provided only on the mounting surface and in the form of flat plates. When the laminated coil component 100 is mounted onto a circuit board, if air is trapped in the solder, it is caught between the external electrodes 130 and the lands, so that it cannot escape from the solder. In this manner, when air remains in the solder, there might be poor connections between the lands and the external electrodes 130.

Therefore, the electronic component 10 has the formation areas A1 and A2 curved so as to bulge at the center relative to the opposite ends in a plan view in the x-axis direction, as shown in FIG. 4. As a result, the external electrodes 14a and 14b, when viewed in a plan view in the x-axis direction,

are also curved so as to bulge at the center toward the negative side in the z-axis direction relative to the opposite ends. Accordingly, when the external electrodes **14a** and **14b** are soldered to the lands, the gap between the lands and the opposite ends of the external electrodes **14a** and **14b** in the y-axis direction is greater than the gap between the lands and the centers of the external electrodes **14a** and **14b** in the y-axis direction. Therefore, even if air is caught between the lands and the external electrodes **14a** and **14b**, it can escape from the solder readily. As a result, the electronic component **10** renders it possible to inhibit air from being left trapped in the solder that connects the lands of the circuit board and the external electrodes **14a** and **14b**.

Furthermore, the electronic component **10** prevents itself from being mounted on the circuit board in a tilted state. More specifically, in the electronic component **10**, the formation areas **A1** and **A2**, when viewed in a plan view in the x-axis direction, are curved so as to bulge at the center relative to the opposite ends, as shown in FIG. 4. As a result, the external electrodes **14a** and **14b**, when viewed in a plan view in the x-axis direction, are also curved so as to bulge at the center toward the negative side in the z-axis direction relative to the opposite ends. Accordingly, when the external electrodes **14a** and **14b** are soldered to the lands, the gap between the lands and the opposite ends of the external electrodes **14a** and **14b** in the y-axis direction is greater than the gap between the lands and the centers of the external electrodes **14a** and **14b** in the y-axis direction. That is, the electronic component **10** has more solder between the lands and the opposite ends of the external electrodes **14a** and **14b** in the y-axis direction when compared to solder between the lands and the external electrodes in an electronic component whose mounting surface is not curved. Accordingly, the surface tension of the solder that pulls the external electrodes **14a** and **14b** toward the circuit board in the electronic component **10** is greater than the surface tension of the solder that pulls the external electrodes toward the circuit board in an electronic component whose mounting surface is not curved. Therefore, the external electrodes **14a** and **14b** are stably attached to the lands. As a result, the electronic component **10** is prevented from being mounted on the circuit board in a tilted state.

The electronic component **10** has features as will be described below to have the bottom surface **S1** curved in a plan view in the x-axis direction. More specifically, the degree of contraction of the insulator layers **16a** to **16j**, which are made of ceramic, is greater than the degree of contraction of the coil conductors **18a** to **18d**, the dummy lead-out conductors **20a** to **20g** and **24a** to **24g**, and the lead-out conductors **22** and **26**, which are made of conductive materials. The proportion of an area occupied by the lead-out conductor **22**, or **26**, and the dummy lead-out conductors **22a** to **22g**, or **24a** to **24g**, in the cross-sectional region **E1** is greater than the proportion of an area occupied by the coil conductors **18a** to **18d** in the cross-sectional region **E2**, as shown in FIG. 4. Accordingly, the cross-sectional region **E2**, which has a relatively small proportion of conductive material, contracts more than the cross-sectional region **E1**, which has a relatively large proportion of conductive material. Accordingly, the width of the cross-sectional region **E2** in the y-axis direction is less than the width of the cross-sectional region **E1** in the y-axis direction, as shown in FIG. 4. Therefore, the opposite ends of the cross-sectional region **E2** in the y-axis direction are pulled upward in the z-axis direction. As a result, the bottom surface **S1** is curved so as to bulge at the center toward the negative side in the z-axis direction relative to the opposite ends.

Furthermore, in the electronic component **10**, the dummy lead-out conductors **20a**, **20b**, **24a**, and **24b** and the dummy lead-out conductors **20f**, **20g**, **24f**, and **24g** are provided outside in the y-axis direction (i.e., either on the positive side or the negative side in the y-axis direction) relative to the terminals **t1** and **t2** of the coil **L**. Accordingly, there is a more significant difference in the degree of contraction in the y-axis direction between the cross-sectional regions **E1** and **E2**. As a result, in the electronic component **10**, the bottom surface **S1** has a larger amount of curving **D**.

Furthermore, the width of the cross-sectional region **E1** in the y-axis direction is larger by the thickness of the dummy lead-out conductors **20a** and **20b**, or **24a** and **24b**, and the dummy lead-out conductors **20f** and **20g**, or **24f** and **24g**. Accordingly, there is an increase in the difference between the width of the cross-sectional region **E1** in the y-axis direction and the width of the cross-sectional region **E2** in the y-axis direction. Therefore, the opposite ends of the cross-sectional region **E2** in the y-axis direction are more strongly pulled upward in the z-axis direction. As a result, in the electronic component **10**, the bottom surface **S1** has a larger amount of curving **D**.

Furthermore, in the electronic component **10**, the dummy lead-out conductors **20c** to **20e** and **24c** to **24e** are provided inside in the y-axis direction relative to the terminals **t1** and **t2** of the coil **L**. Accordingly, there is a more significant difference in the degree of contraction in the y-axis direction between the cross-sectional regions **E1** and **E2**. As a result, in the electronic component **10**, the bottom surface **S1** has a larger amount of curving **D**.

Furthermore, in the electronic component **10**, the lead-out conductors **22** and **26** and the dummy lead-out conductors **20a** to **20f** and **24a** to **24f** are thicker than the coil conductors **18a** to **18d**, as shown in FIG. 4. Therefore, the proportion of an area occupied by the lead-out conductor **22**, or **26**, and the dummy lead-out conductors **22a** to **22g**, or **24a** to **24g**, in the cross-sectional region **E1** can be rendered greater than the proportion of an area occupied by the coil conductors **18a** to **18d** in the cross-sectional region **E2**. As a result, in the electronic component **10**, the bottom surface **S1** has a larger amount of curving **D**.

To clearly demonstrate that the electronic component **10** is prevented from being mounted on the circuit board in a tilted state, the present inventor conducted the experimentation as will be described below. FIG. 5 is a diagram illustrating an electronic component **10** mounted on a circuit board **200**.

The present inventor produced electronic components **10** with specifications shown below as first through fourteenth samples, with one electronic component for each sample. Table 1 shows the amount of curving **D** for each of the first through fourteenth samples. The amounts of curving **D** were measured by the length measurement function of a digital microscope VHX-500 from KEYENCE Corp. after observing cross sections of the first through fourteenth samples at a magnification of 500 times using the microscope.

Chip size: 0603 size (0.6 mm×0.3 mm)

Electrode size: 0.15 mm×0.28 mm

TABLE 1

| AMOUNT OF CURVING D(μm) |      |
|-------------------------|------|
| 1ST SAMPLE              | 0.08 |
| 2ND SAMPLE              | 0.15 |
| 3RD SAMPLE              | 0.23 |
| 4TH SAMPLE              | 0.57 |
| 5TH SAMPLE              | 0.98 |
| 6TH SAMPLE              | 1.88 |
| 7TH SAMPLE              | 3.25 |
| 8TH SAMPLE              | 3.99 |

## 11

TABLE 1-continued

| AMOUNT OF CURVING D(μm) |       |
|-------------------------|-------|
| 9TH SAMPLE              | 6.91  |
| 10TH SAMPLE             | 8.14  |
| 11TH SAMPLE             | 11.75 |
| 12TH SAMPLE             | 12.5  |
| 13TH SAMPLE             | 15.15 |
| 14TH SAMPLE             | 18.25 |

The present inventor mounted the first through fourteenth samples onto circuit boards 200 by joining external electrodes 14a and 14b to lands 202 with solder 300, as shown in FIG. 5. Thereafter, the inclination  $\theta$  of the electronic component 10 relative to the circuit board 200 was measured. The inclination  $\theta$  is an angle of a normal to the bottom surface S1 with respect to a normal to the circuit board 200, as shown in FIG. 5. The inclination  $\theta$  was measured by a CNC video measuring system NEXIV (model: VMR-3020, manufactured by Nikon Corp.). Table 2 shows the experimentation results.

TABLE 2

| INCLINATION $\theta$ (°) |     |
|--------------------------|-----|
| 1ST SAMPLE               | 5.9 |
| 2ND SAMPLE               | 4.9 |
| 3RD SAMPLE               | 4.6 |
| 4TH SAMPLE               | 3.3 |
| 5TH SAMPLE               | 2.5 |
| 6TH SAMPLE               | 2.3 |
| 7TH SAMPLE               | 2.2 |
| 8TH SAMPLE               | 2   |
| 9TH SAMPLE               | 1.8 |
| 10TH SAMPLE              | 1.6 |
| 11TH SAMPLE              | 1.7 |
| 12TH SAMPLE              | 1.7 |
| 13TH SAMPLE              | 1.7 |
| 14TH SAMPLE              | 1.8 |

From Table 2, it can be appreciated that the inclination  $\theta$  decreases as the amount of curving D increases. Thus, it can be appreciated that curving the bottom surface S1 prevents the electronic component 10 from being mounted on the circuit board 200 in a tilted state.

Furthermore, after the mounting of the electronic component 10, a visual inspection is carried out through image processing in order to confirm whether the electronic component 10 is mounted at a normal position and with a normal attitude. At this time, if the inclination  $\theta$  is 5° or more, the side surface S3 or the side surface S4 of the electronic component 10, along with the top surface S2, is measured so that the electronic component 10 is determined to be mounted poorly. Therefore, the inclination  $\theta$  is preferably less than 5°. The inclination  $\theta$  for the first sample with an amount of curving D of 0.08 μm was 5.9°, and the inclination  $\theta$  for the second sample with an amount of curving D of 0.15 μm was 4.9°. Accordingly, the amount of curving D is preferably 0.15 μm or more.

Furthermore, given that the electronic component 10 is sucked by a nozzle, the amount of curving D is preferably 12.5 μm or less. FIGS. 6A and 6B are diagrams each illustrating the electronic component 10 sucked by a nozzle 600.

The electronic component 10 is affixed to a taping mount 500, as shown in FIG. 6A. In mounting the electronic component 10, the electronic component 10 is sucked at the top surface S2 by the nozzle 600, and detached from the taping mount 500.

## 12

Here, if the amount of curving D of the bottom surface S1 is excessively increased, the electronic component 10 might be tilted on the taping mount 500, as shown in FIG. 6B. As a result, it might be difficult to suck the top surface S2 of the electronic component 10 by the nozzle 600. In the experimentation by the present inventor, there was no suction error for the twelfth sample having an amount of curving D of 12.5 but a suction error occurred for the thirteenth sample having an amount of curving D of 15.15 μm. Therefore, from 10 the viewpoint of preventing a suction error, the amount of curving D is preferably 12.5 μm or less.

First Modification: Hereinafter, an electronic component 10a according to a first exemplary modification will be described with reference to the drawings. FIG. 7 is a cross-sectional structure view of the electronic component 10a according to the first modification. For the external oblique view of the electronic component 10a, FIG. 3 will be referenced.

In the electronic component 10a, the thickness T2 of the dummy lead-out conductors 20a, 20b, 20f, 20g, 24a, 24b, 24f, and 24g provided outside in the y-axis direction relative to the terminals t1 and t2 of the coil L is greater than the thickness T1 of the dummy lead-out conductors 20c to 20e and 24c to 24e and the lead-out conductors 22 and 26 provided inside in the y-axis direction relative to the terminals t1 and t2. In addition, the thickness of the coil conductors 18a to 18d is equal to the thickness T1 of the dummy lead-out conductors 20c to 20e and 24c to 24e and the lead-out conductors 22 and 26.

In the electronic component 10a as above, the thickness T2 of the dummy lead-out conductors 20a, 20b, 20f, 20g, 24a, 24b, 24f, and 24g is greater than the thickness T1 of the coil conductors 18a to 18d. Accordingly, the proportion of an area occupied by the lead-out conductor 22, or 26, and the dummy lead-out conductors 22a to 22g, or 24a to 24g, in the cross-sectional region E1 can be rendered greater than the proportion of an area occupied by the coil conductors 18a to 18d in the cross-sectional region E2. As a result, in the electronic component 10a, the bottom surface S1 has a larger amount of curving D.

Furthermore, in the electronic component 10a, the dummy lead-out conductors 20c to 20e and 24c to 24e and the lead-out conductors 22 and 26 have the same thickness T1 as the coil conductors 18a to 18d. Accordingly, among the dummy lead-out conductors 20c to 20e and 24c to 24e, the lead-out conductors 22 and 26, and the coil conductors 18a to 18d, any conductors that are to be formed on the same insulator layer 16 can be formed simultaneously by screen printing. As a result, the number of production steps for the electronic component 10a can be reduced.

Second Modification: Hereinafter, an electronic component 10b according to a second exemplary modification will be described with reference to the drawings. FIG. 8 is a cross-sectional structure view of the electronic component 10b according to the second modification. For the external oblique view of the electronic component 10b, FIG. 3 will be referenced.

In the electronic component 10b, the thickness T4 of the insulator layers 16a to 16c and 16g to 16j provided outside in the y-axis direction relative to the terminals t1 and t2 of the coil L is less than the thickness T3 of the insulator layers 16d to 16f provided inside in the y-axis direction relative to the terminals t1 and t2.

In the electronic component 10b as above, since the thickness T4 of the insulator layers 16a to 16c, 16g to 16j is small, the proportion of an area occupied by the dummy lead-out conductors 20a, 20b, 20e, and 20f, or 24a, 24b, 24e,

## 13

and 24f, outside the terminals t1 and t2 of the coil L within the cross-sectional region E1 increases. Accordingly, portions outside the terminals t1 and t2 of the coil L within the cross-sectional region E1 become more resistant to contraction. As a result, in the electronic component 10b, the bottom surface S1 has a larger amount of curving D.

Third Modification: Hereinafter, an electronic component 10c according to a third exemplary modification will be described with reference to the drawings. FIG. 9 is a cross-sectional structure view of the electronic component 10c according to the third modification. For the external oblique view of the electronic component 10c, FIG. 3 will be referenced.

In the electronic component 10c, the height from the bottom surface S1 to the top of the dummy lead-out conductors 20a, 20b, 20f, 20g, 24a, 24b, 24f, and 24g provided outside in the y-axis direction relative to the terminals t1 and t2 of the coil L is higher than the height from the bottom surface S1 to the top of the dummy lead-out conductors 20c to 20e and 24c to 24e and the lead-out conductors 22 and 26 provided inside in the y-axis direction relative to the terminals t1 and t2.

Also in the electronic component 10c as above, the proportion of an area occupied by the dummy lead-out conductors 20a, 20b, 20e, and 20f, or 24a, 24b, 24e, and 24f, outside the terminals t1 and t2 of the coil L within the cross-sectional region E1 increases. Accordingly, portions outside the terminals t1 and t2 of the coil L within the cross-sectional region E1 become more resistant to contraction. As a result, in the electronic component 10c, the bottom surface S1 has a larger amount of curving D.

Fourth Modification: Hereinafter, an electronic component 10d according to a fourth exemplary modification will be described with reference to the drawings. FIG. 10A is an external oblique view of a laminate 12 in the electronic component 10d according to the fourth modification. FIG. 10B is an external oblique view of the electronic component 10d according to the fourth modification.

In the electronic component 10d, the lead-out conductor 22 and the dummy lead-out conductors 20a to 20g are exposed at the end surface S6. As a result, the external electrode 14a extends in an L-like shape across the bottom surface S1 and the end surface S6.

Furthermore, the lead-out conductor 26 and the dummy lead-out conductors 24a to 24g are exposed at the end surface S5. As a result, the external electrode 14b extends in an L-like shape across the bottom surface S1 and the end surface S5.

In the electronic component 10d as above, solder adheres to the part of the external electrode 14a that is provided on the side surface S6 and the part of the external electrode 14b that is provided on the side surface S5. Accordingly, the surface tension of the solder that pulls the electronic component 10d toward the circuit board is greater than the surface tension of the solder that pulls the electronic component 10 toward the circuit board. As a result, the electronic component 10d can be mounted on the circuit board more firmly.

Note that the external electrodes 14a and 14b may be formed so as to extend to the side surfaces S3 and S4, as well.

Fifth Modification: Hereinafter, an electronic component 10e according to a fifth exemplary modification will be described with reference to the drawings. FIGS. 11A, 11B, and 11C are plan views of the electronic component 10e according to the fifth modification. FIG. 12 is an exploded view of a laminate 12 in the electronic component 10e

## 14

according to the fifth modification. FIG. 13A is an external oblique view of the laminate 12 in the electronic component 10e according to the fifth modification. FIG. 13B is an external oblique view of the electronic component 10e according to the fifth modification. FIG. 14 is a cross-sectional structure view taken along line X-X of FIG. 13A. In FIG. 14, external electrodes 14a and 14b are not shown. In the following, the direction of lamination of the electronic component 10e will be defined as an x-axis direction, the top-bottom direction in a plan view in the x-axis direction will be defined as a z-axis direction, and the left-right direction in a plan view in the x-axis direction will be defined as a y-axis direction. The x-, y-, and z-axes are perpendicular to one another.

The electronic component 10e includes the laminate 12, the external electrodes 14a and 14b, dummy lead-out conductors 20a, 20b, 24a, and 24b, lead-out conductors 22 and 26, a coil L, and via-hole conductors v4 to v9, as shown in FIGS. 11A, 11B, 11C, and 12.

The laminate 12 is in the shape of a rectangular solid, and has the coil L provided therein. The laminate 12 has a bottom surface S1, a top surface S2, side surfaces S3 and S4, and end surfaces S5 and S6. The bottom surface S1 is a surface of the laminate 12 on the negative side in the y-axis direction, and serves as a mounting surface to face a circuit board when the electronic component 10e is mounted on the circuit board. The top surface S2 is a surface of the laminate 12 on the positive side in the z-axis direction. The side surface S3 is a surface of the laminate 12 on the negative side in the x-axis direction. The side surface S4 is a surface of the laminate 12 on the positive side in the x-axis direction. The end surface S5 is a surface of the laminate 12 on the negative side in the y-axis direction. The end surface S6 is a surface of the laminate 12 on the positive side in the y-axis direction.

The laminate 12 is formed by laminating insulator layers 16a to 16l in this order, from the positive side toward the negative side in the x-axis direction, as shown in FIG. 12. Each of the insulator layers 16a to 16l has a square shape, and is made of, for example, a Ni—Cu—Zn ferrite magnetic material. In the following, the surfaces of the insulator layers 16a to 16l on the positive side in the x-axis direction will be referred to as the front faces, and the surfaces of the insulator layers 16a to 16l on the negative side in the x-axis direction will be referred to as the back faces.

The bottom surface S1 is formed by a series of the sides of the insulator layers 16a to 16l on the negative side in the z-axis direction. The top surface S2 is formed by a series of the sides of the insulator layers 16a to 16l on the positive side in the z-axis direction. The side surface S3 is formed by the back face of the insulator layer 16l. The side surface S4 is formed by the front face of the insulator layer 16a. The end surface S5 is formed by a series of the sides of the insulator layers 16a to 16l on the negative side in the y-axis direction. The end surface S6 is formed by a series of the sides of the insulator layers 16a to 16l on the positive side in the y-axis direction.

The coil L includes coil conductors 18a to 18d and via-hole conductors v1 to v3, as shown in FIG. 12. The coil L is a helical coil formed by connecting the coil conductors 18a to 18d by the via-hole conductors v1 to v3. The coil L has a coil axis extending in the x-axis direction, and spirals counterclockwise toward the negative side in the x-axis direction in a plan view from the positive side in the x-axis direction. Moreover, the coil L has terminals t1 and t2. The terminal t1 of the coil L is positioned on the positive side in the x-axis direction relative to the terminal t2.

## 15

The coil conductors **18a** to **18d** are provided on the insulator layers **16e** to **16h**, respectively, as shown in FIG. 12. Each of the coil conductors **18a** to **18d** is made of an Ag-based conductive material, and is a linear conductor curved in a U-like shape. Moreover, the coil conductors **18a** to **18d** overlap one another to form a square in a plan view in the x-axis direction. In the following, the ends of the coil conductors **18a** to **18d** that are located upstream in the counterclockwise direction will be simply referred to as the upstream ends, and the ends of the coil conductors **18a** to **18d** that are located downstream in the counterclockwise direction will be simply referred to as the downstream ends. The terminal **t1** of the coil **L** is at the upstream end of the coil conductor **18a**, and the terminal **t2** of the coil **L** is at the downstream end of the coil conductor **18d**.

The via-hole conductors **v1** to **v3** connect the coil conductors **18a** to **18d**. More specifically, the via-hole conductor **v1** connects the downstream end of the coil conductor **18a** to the upstream end of the coil conductor **18b**. The via-hole conductor **v2** connects the downstream end of the coil conductor **18b** to the upstream end of the coil conductor **18c**. The via-hole conductor **v3** connects the downstream end of the coil conductor **18c** to the upstream end of the coil conductor **18d**.

The lead-out conductor **22** is provided on the front face of the insulator layer **16d**, so as to be exposed between the insulator layers **16c** and **16d** at the bottom surface **S1** and the end surfaces **S5** and **S6**. More specifically, the lead-out conductor **22** has a rectangular shape extending in the y-axis direction and provided along the side of the insulator layer **16d** on the negative side in the z-axis direction, and the lead-out conductor **22** is in contact with opposite ends of the insulator layer **16d** in the y-axis direction. As a result, the lead-out conductor **22** is exposed at the bottom surface **S1** as a linear strip extending in the y-axis direction, and also exposed at the end surfaces **S5** and **S6** as a linear strip extending in the z-axis direction.

The dummy lead-out conductors **20a** and **20b** are provided on the front faces of the insulator layers **16b** and **16c**, respectively, so as to be exposed between the insulator layers **16a** to **16c** at the bottom surface **S1**. The dummy lead-out conductors **20a** and **20b** have the same shape as the lead-out conductor **22**, and are aligned in an entirely overlapping manner in a plan view in the y-axis direction. As a result, the lead-out conductor **22** and the dummy lead-out conductors **20a** and **20b** are exposed within a rectangular formation area **A1** at the bottom surface **S1**, as shown in FIG. 13A.

The lead-out conductor **26** is provided on the front face of the insulator layer **16i**, so as to be exposed between the insulator layers **16h** and **16i** at the bottom surface **S1** and the end surfaces **S5** and **S6**. More specifically, the lead-out conductor **26** has a rectangular shape extending in the y-axis direction and provided along the side of the insulator layer **16i** on the negative side in the z-axis direction, and the lead-out conductor **26** is in contact with opposite ends of the insulator layer **16i** in the y-axis direction. As a result, the lead-out conductor **26** is exposed at the bottom surface **S1** as a linear strip extending in the y-axis direction, and also exposed at the end surfaces **S5** and **S6** as a linear strip extending in the z-axis direction.

The dummy lead-out conductors **24a** and **24b** are provided on the front faces of the insulator layers **16j** and **16k**, respectively, so as to be exposed between the insulator layers **16i** to **16k** at the bottom surface **S1**. The dummy lead-out conductors **24a** and **24b** have the same shape as the lead-out conductor **26**, and are aligned in an entirely overlapping manner in a plan view in the y-axis direction. As a result, the

## 16

lead-out conductor **26** and the dummy lead-out conductors **24a** and **24b** are exposed within a rectangular formation area **A2** at the bottom surface **S1**, as shown in FIG. 13A.

The via-hole conductors **v4** to **v6** are provided so as to pierce through the insulator layers **16b** to **16d**, respectively, in the x-axis direction, and overlap one another in a plan view in the x-axis direction. The via-hole conductor **v4** connects the dummy lead-out conductors **20a** and **20b**. The via-hole conductor **v5** connects the dummy lead-out conductor **20b** and the lead-out conductor **22**. The via-hole conductor **v6** connects the lead-out conductor **22** and the upstream end of the coil conductor **18a**.

The via-hole conductors **v7** to **v9** are provided so as to pierce through the insulator layers **16h** to **16j**, respectively, in the x-axis direction, and overlap one another in a plan view in the x-axis direction. The via-hole conductor **v7** connects the downstream end of the coil conductor **18d** and the lead-out conductor **26**. The via-hole conductor **v8** connects the lead-out conductor **26** and the dummy lead-out conductor **24a**. The via-hole conductor **v9** connects the dummy lead-out conductors **24a** and **24b**.

The external electrode **14a** is formed by directly plating the bottom surface **S1** and the end surfaces **S5** and **S6**, so as to cover the dummy lead-out conductors **20a** and **20b** and the lead-out conductor **22**, as shown in FIG. 13B. As a result, the external electrode **14a** is formed within the formation area **A1** at the bottom surface **S1** of the laminate **12**. The external electrode **14b** is formed by directly plating the bottom surface **S1** and the end surfaces **S5** and **S6**, so as to cover the dummy lead-out conductors **24a** and **24b** and the lead-out conductor **26**, as shown in FIG. 13B. As a result, the external electrode **14b** is formed within the formation area **A2** at the bottom surface **S1** of the laminate **12**. Moreover, the external electrode **14a** is positioned on the positive side in the x-axis direction relative to the external electrode **14b**. Examples of the materials of the external electrodes **14a** and **14b** include Cu, Ni, and Sn.

The electronic component **10e** thus configured has features as will be described below, in the cross section shown in FIG. 14, which is normal to the y-axis direction and includes the lead-out conductor **22**, the dummy lead-out conductors **20a** and **20b**, and the coil conductors **18a** to **18d**. First, a portion of the cross section that includes the lead-out conductor **22** and the dummy lead-out conductors **20a** to **20g** will be referred to as a cross-sectional region **E1**. The rest of the cross section other than the cross-sectional region **E1**, which includes the coil conductors **18a** to **18d**, will be referred to as a cross-sectional region **E2**. The cross-sectional region **E1** is a region between the bottom surface **S1** and a line **L2** parallel to the x-axis and dividing the dummy lead-out conductors **20a** to **20g** from the coil conductors **18a** to **18d**. The cross-sectional region **E2** is a region between the top surface **S2** and the line **L2**.

As shown in FIG. 14, the proportion of an area occupied by the lead-out conductor **22** and the dummy lead-out conductors **20a** and **20b** in the cross-sectional region **E1** is greater than the proportion of an area occupied by the coil conductors **18a** to **18d** in the cross-sectional region **E2**.

Furthermore, there are features as will be described below, in a cross section normal to the y-axis direction and including the lead-out conductor **26**, the dummy lead-out conductors **24a** and **24b**, and the coil conductors **18a** to **18d**. First, a portion of the cross section that includes the lead-out conductor **26** and the dummy lead-out conductors **24a** and **24b** will be referred to as a cross-sectional region **E1**. The rest of the cross section other than the cross-sectional region **E1**, which includes the coil conductors **18a** to **18d**, will be

referred to as a cross-sectional region E2. The cross-sectional region E1 is a region between the bottom surface S1 and a line L2 parallel to the x-axis and dividing the coil conductors 18a to 18d from the dummy lead-out conductors 24a and 24b. The cross-sectional region E2 is a region between the top surface S2 and the line L2.

The proportion of an area occupied by the lead-out conductor 26 and the dummy lead-out conductors 24a and 24b in the cross-sectional region E1 is greater than the proportion of an area occupied by the coil conductors 18a to 18d in the cross-sectional region E2.

Furthermore, in the electronic component 10e, the formation areas A1 and A2, when viewed in a plan view in an extending direction (y-axis direction) in which the sides of the insulator layers 16a to 16l that constitute the bottom surface S1 extend, are curved so as to bulge at the center toward the negative side in the z-axis direction relative to the opposite ends, as shown in FIG. 14.

Furthermore, the external electrodes 14a and 14b are provided in the formation areas A1 and A2, respectively. Therefore, the external electrodes 14a and 14b, when viewed in a plan view in the y-axis direction, are also curved so as to bulge at the center toward the negative side in the z-axis direction relative to the opposite ends.

As with the electronic component 10, the electronic component 10e thus configured renders it possible to inhibit air from being left trapped in the solder that connects the lands of the circuit board to the external electrodes 14a and 14b.

Furthermore, in the electronic component 10e, solder adheres to the parts of the external electrode 14a that are provided at the end surfaces S5 and S6 and the parts of the external electrode 14b that are provided at the end surfaces S5 and S6. Accordingly, the surface tension of the solder that pulls the electronic component 10e toward the circuit board is greater than the surface tension of the solder that pulls the electronic component 10 toward the circuit board. As a result, the electronic component 10e can be mounted on the circuit board more firmly.

Furthermore, in the electronic component 10e, the external electrodes 14a and 14b are not provided at the side surfaces S3 and S4. Therefore, an eddy-current loss is inhibited from being caused by the passage of a magnetic flux generated by the coil L, so that a reduction in the Q factor of the coil L is inhibited.

Furthermore, the axis of the coil L is perpendicular to the side surfaces S3 and S4, and the external electrodes 14a and 14b are not provided at the side surfaces S3 and S4. Accordingly, there is less floating capacitance between the coil L and the external electrodes 14a and 14b. As a result, the high-frequency characteristics of the coil L are improved.

#### OTHER EMBODIMENTS

The present disclosure is not limited to the electronic components 10 and 10a to 10e, and modifications can be made within the spirit and scope of the disclosure.

Note that the dummy lead-out conductors 20 and 24 are not necessarily connected by via-hole conductors.

Note that in the electronic component 10, the coil conductors 18a to 18d, the dummy lead-out conductors 20a to 20g and 24a to 24g, and the lead-out conductors 22 and 26 may be equal in thickness.

Note that the circuit elements included in the electronic components 10 and 10a to 10e are not limited to the coils L. Accordingly, the circuit elements may be capacitors, etc.

Note that the features of the electronic components 10 and 10a to 10e may be provided in combination.

Although the present disclosure has been described in connection with the preferred embodiment above, it is to be noted that various changes and modifications are possible to those who are skilled in the art. Such changes and modifications are to be understood as being within the scope of the disclosure.

What is claimed is:

1. An electronic component comprising:  
a laminate having a plurality of rectangular insulator layers and a mounting surface formed by a series of sides of the insulator layers;  
a plurality of first lead-out conductors exposed between the insulator layers at the mounting surface;  
a first external electrode covering the first lead-out conductors at the mounting surface;  
a plurality of second lead-out conductors exposed between the insulator layers at the mounting surface;  
and  
a second external electrode covering the second lead-out conductors at the mounting surface,  
the first external electrode being located at a first formation area at the mounting surface, and  
the first formation area, when viewed in a plan view in an extending direction in which the sides of the insulator layers that constitute the mounting surface extend, being curved so as to bulge at a center of the first formation area relative to opposite ends thereof.

2. The electronic component according to claim 1, further comprising a circuit element including a plurality of conductive members.

3. The electronic component according to claim 2, wherein,

- in a cross section normal to the extending direction and including the first lead-out conductors and the conductive members, a part of the cross section is a first cross-sectional region including the first lead-out conductors and the mounting surface, and the rest of the cross section other than the first cross-sectional region is a second cross-sectional region including the conductive members,  
a proportion of an area occupied by the first lead-out conductors in the first cross-sectional region is greater than the proportion of an area occupied by the conductive members in the second cross-sectional region.

4. The electronic component according to claim 2, wherein a part of the first lead-out conductors is provided outside of opposite ends of the circuit element in a direction of lamination of the plurality of rectangular insulator layers.

5. The electronic component according to claim 4, wherein the part of the first lead-out conductor provided outside the opposite ends of the circuit element is thicker than the first lead-out conductor provided inside the opposite ends of the circuit element in the direction of lamination.

6. The electronic component according to claim 4, wherein a height from the mounting surface to a top of one first lead-out conductor provided outside the opposite ends of the circuit element in the direction of lamination is greater than a height from the mounting surface to a top of one first lead-out conductor provided inside the opposite ends of the circuit element in the direction of lamination.

7. The electronic component according to claim 2, wherein each of the first lead-out conductors is thicker than each of the conductive members.

8. The electronic component according to claim 2, wherein one insulator layer provided outside opposite ends

## 19

of the circuit element in a direction of lamination of the plurality of rectangular insulator layers is thinner than one insulator layer provided inside the opposite ends of the circuit element in the direction of lamination.

9. The electronic component according to claim 1, wherein the first external electrode and the second external electrode are arranged in the extending direction.

10. The electronic component according to claim 9, wherein, in a plan view in the extending direction, a distance in a direction normal to the mounting surface from the most bulging point of the mounting surface to the opposite ends of the mounting surface is from 0.15  $\mu\text{m}$  to 12.5  $\mu\text{m}$ .

11. The electronic component according to claim 1, wherein the first external electrode is formed by plating.

12. The electronic component according to claim 1, wherein the laminate is sintered.

13. The electronic component according to claim 1, wherein

the second external electrode is located at a second formation area at the mounting surface, and the second formation area, when viewed in a plan view in the extending direction, is curved so as to bulge at a center of the second formation area relative to opposite ends thereof.

14. A method for producing an electronic component including a laminate having a plurality of rectangular insulator layers and a mounting surface formed by a series of sides of the insulator layers;

a plurality of first lead-out conductors exposed between the insulator layers at the mounting surface;

a first external electrode covering the first lead-out conductors at the mounting surface;

a plurality of second lead-out conductors exposed between the insulator layers at the mounting surface; and

a second external electrode covering the second lead-out conductors at the mounting surface,

the first external electrode being located at a first formation area at the mounting surface, and

the first formation area, when viewed in a plan view in an extending direction in which the sides of the insulator layers that constitute the mounting surface extend, being curved so as to bulge at a center of the first formation area relative to opposite ends thereof, and a circuit element including a plurality of conductive members, comprising steps of:

obtaining the laminate in an unfired state, the laminate being provided with the first lead-out conductors and the conductive members; and

firing the laminate.

15. An electronic component comprising:

a laminate having a plurality of rectangular insulator layers and a mounting surface formed by a series of sides of the insulator layers,

a plurality of first lead-out conductors exposed between the insulator layers at the mounting surface,

a first external electrode covering the first lead-out conductors at the mounting surface,

a plurality of second lead-out conductors exposed between the insulator layers at the mounting surface,

a second external electrode covering the second lead-out conductors at the mounting surface,

the first external electrode being provided in a first formation area at the mounting surface, and

the first formation area, when viewed in a plan view in an extending direction in which the sides of the insulator layers that constitute the mounting surface extend,

5

## 20

being curved so as to bulge at a center relative to opposite ends of the first formation area, a second formation area, when viewed in the plan view, being curved so as to bulge at a center relative to opposite ends of the second formation area.

16. The electronic component according to claim 15, further comprising a circuit element including a plurality of conductive members.

17. An electronic component comprising:

a laminate having a plurality of rectangular insulator layers and a mounting surface formed by a series of sides of the insulator layers;

a plurality of first lead-out conductors exposed between the insulator layers at the mounting surface; and a first external electrode covering the first lead-out conductors at the mounting surface,

the first external electrode being located at a first formation area at the mounting surface, and the first formation area, when viewed in a plan view in an extending direction in which the sides of the insulator layers that constitute the mounting surface extend, being curved so as to bulge at a center of the first formation area relative to opposite ends thereof, wherein

in a cross section normal to the extending direction and including the first lead-out conductors and the conductive members, a part of the cross section is a first cross-sectional region including the first lead-out conductors and the mounting surface, and the rest of the cross section other than the first cross-sectional region is a second cross-sectional region including the conductive members,

a proportion of an area occupied by the first lead-out conductors in the first cross-sectional region is greater than the proportion of an area occupied by the conductive members in the second cross-sectional region.

18. An electronic component comprising:

a laminate having a plurality of rectangular insulator layers and a mounting surface formed by a series of sides of the insulator layers;

a plurality of first lead-out conductors exposed between the insulator layers at the mounting surface;

a first external electrode covering the first lead-out conductors at the mounting surface,

the first external electrode being located at a first formation area at the mounting surface, and

the first formation area, when viewed in a plan view in an extending direction in which the sides of the insulator layers that constitute the mounting surface extend, being curved so as to bulge at a center of the first formation area relative to opposite ends thereof; and a circuit element including a plurality of conductive members; wherein

a part of the first lead-out conductors is provided outside of opposite ends of the circuit element in a direction of lamination of the plurality of rectangular insulator layers, and the part of the first lead-out conductor provided outside the opposite ends of the circuit element is thicker than the first lead-out conductor provided inside the opposite ends of the circuit element in the direction of lamination.

19. An electronic component comprising:

a laminate having a plurality of rectangular insulator layers and a mounting surface formed by a series of sides of the insulator layers;

50

60

65

**21**

a plurality of first lead-out conductors exposed between the insulator layers at the mounting surface;  
 a first external electrode covering the first lead-out conductors at the mounting surface,  
 the first external electrode being located at a first formation area at the mounting surface, and  
 the first formation area, when viewed in a plan view in an extending direction in which the sides of the insulator layers that constitute the mounting surface extend, being curved so as to bulge at a center of the first formation area relative to opposite ends thereof; and  
 a circuit element including a plurality of conductive members; wherein  
 one insulator layer provided outside opposite ends of the circuit element in a direction of lamination of the plurality of rectangular insulator layers is thinner than one insulator layer provided inside the opposite ends of the circuit element in the direction of lamination. 15  
**20.** An electronic component comprising:  
 a laminate having a plurality of rectangular insulator layers and a mounting surface formed by a series of sides of the insulator layers;  
 a plurality of first lead-out conductors exposed between the insulator layers at the mounting surface; 20

**22**

a first external electrode covering the first lead-out conductors at the mounting surface,  
 the first external electrode being located at a first formation area at the mounting surface, and  
 the first formation area, when viewed in a plan view in an extending direction in which the sides of the insulator layers that constitute the mounting surface extend, being curved so as to bulge at a center of the first formation area relative to opposite ends thereof; and  
 a circuit element including a plurality of conductive members; wherein  
 a part of the first lead-out conductors is provided outside of opposite ends of the circuit element in a direction of lamination of the plurality of rectangular insulator layers, and  
 a height from the mounting surface to a top of one first lead-out conductor provided outside the opposite ends of the circuit element in the direction of lamination is greater than a height from the mounting surface to a top of one first lead-out conductor provided inside the opposite ends of the circuit element in the direction of lamination. 10

\* \* \* \* \*